

## UNITED STATES PATENT OFFICE

2,672,447

OXIDATION RESISTANT TRANSFORMER  
OILS AND THE LIKE

William T. Stewart, Berkeley, Charles D. Newnan,  
San Pablo, and Neal W. Furby, Berkeley, Calif.,  
assignors to California Research Corporation,  
San Francisco, Calif., a corporation of Delaware

No Drawing. Application August 9, 1949,  
Serial No. 109,426

5 Claims. (Cl. 252—63.7)

**1**  
This invention relates to the stabilization of lubricating oil compositions intended for use in the service of transformer oils, turbine oils and the like. More particularly, this invention pertains to mineral oil compositions useful as transformer oils, wherein the anti-oxidation characteristics of the anti-oxidant present in the composition (e. g., selenium compounds) have been enhanced by the presence of hydroxyanthraquinone compounds (e. g., quinizarin).

For a number of years, it has been the general practice to use moderately treated mineral oils as transformer oils. These moderately treated oils, however, gradually deteriorate in service. This deterioration is normally due to oxidation effects, which effects are increased several fold by the presence of the materials (i. e., the brass, copper, silica steel, etc.) of the transformer systems, which materials serve as oxidation catalysts. In turbine oils, the oxidation is catalytically promoted by the copper, lead, steel and brass which are found in the turbine system.

The effectiveness of a transformer oil as an insulating oil is materially reduced by the oxidation products (i. e., the acid products) formed. Furthermore, these acid products gradually attack the insulation on the wires of the transformer system, leaving the wires partially exposed to the oil, which oil then serves as a transmitter of current instead of an inhibitor of current. In the turbine oils the oxidation products (i. e., the acid sludges) corrode the bearings and other parts of the turbine system and clog the oil lines, etc.

It is a tremendous advantage in transformer, turbine, and like systems, to use the oils of sufficient oxidation stability to permit their use over long periods of time without being changed. Not only is it desirable to have transformer oils and the like highly resistant to oxidation, but it is also a desired feature of the transformer oils and the like that the viscosity index be high; that is, that only small changes in viscosity occur with large changes in temperature. Thus, in order to obtain oils of high viscosity index, the base oils are subjected to such effective methods of refining as the selective solvent extraction processes wherein the lower viscosity index hydrocarbons are selectively dissolved. These selective solvent refining processes concentrate in 50 one fraction, usually the undissolved oil fraction, those compounds of a "paraffinic" nature which show a smaller change in viscosity upon change in temperature.

However, highly-refined oils have smaller 55

**2**  
amounts of the naturally occurring oxidation inhibitors present in the oils than do less-refined oils. That is, these naturally occurring inhibitors have been removed at least to an extent which materially reduces the oxidation stability of the oil when used as transformer oils and as turbine oils.

When oxidation inhibitors are added to highly refined oils and oils which are not so highly refined, it is found that the highly refined oils are more responsive to the oxidation inhibitors; that is, when the oxidation inhibitors of this invention are incorporated in so-called over-refined oils, a greater resistance to oxidation is obtained than when the oxidation inhibitors are used in conjunction with a less-refined lubricating oil.

In attempting to increase the oxidation stability of transformers and turbine oils, known oxidation inhibitors (such as the dialkyl selenides of Denison and Condit Patents 2,398,414 and 2,398,415) were incorporated therein, and, as expected, the resulting compounded oils were more resistant to oxidation than the base oils containing no inhibitors. However, it was not to be expected that the oxidation stability of the oil thus compounded with oxidation inhibitors could be increased still further by adding thereto an agent which by itself is not an oxidation inhibitor.

It is an outstanding feature of this invention that the oxidation stability of a lubricating oil compounded with an oxidation inhibitor is materially increased by adding thereto an agent not known as an oxidation inhibitor which agent asserts synergistic effects in combination with the oxidation inhibitors of this invention.

It is a primary object of this invention to produce lubricating oil compositions which are highly resistant to oxidation.

It is another object of this invention to incorporate in mineral oils containing oxidation inhibitors an agent exhibiting a marked synergistic effect on certain oxidation inhibitors.

It is a further object of this invention to produce transformer oils and the like which are more resistant to oxidation than those heretofore known.

These and other objects may be obtained from the disclosures and the claims noted hereinbelow.

It has been discovered that highly oxidation resistant compositions of oils of lubricating viscosity may be prepared by incorporating hydroxy anthraquinones in said compositions containing oxidation inhibitors, particularly, selenides.

The hydroxy anthraquinones of this invention

are anthraquinones containing two hydroxyl groups on the ring, such as exemplified by alizarin (1,2-dihydroxy-anthraquinone), quinizarin (1,4-dihydroxy-anthraquinone), 1,5-dihydroxy-anthraquinone and 1,8-dihydroxyanthraquinone. It is preferred to use dihydroxy anthraquinones particularly, quinizarin.

Oxidation inhibitors which are contemplated by this invention to be used in viscous oil compositions in combination with hydroxy-anthraquinones include selenides. The particular selenides of the present invention may be represented by the formula:



wherein A is R<sub>1</sub>, Se—R<sub>2</sub>, M or a hydrogen atom, R, R<sub>1</sub> and R<sub>2</sub> are like or unlike substantially-hydrocarbonaceous organo groups connected to selenium through an aliphatic carbon atom, at least R, and preferably also R<sub>1</sub> and R<sub>2</sub>, contain at least 10 carbon atoms, preferably 12 to 30 carbon atoms, and M represents a cationic salt-forming radical, such as a metal atom. Thus, the selenides embrace di-organo mono- and diselenides, selenomercaptans (organo hydroselenides) and selenomercaptides (metallo organo selenides). Preferred are the di-organo selenides (i. e., R'—Se—R'', where n=1 or 2 and R' and R'' are like or unlike aliphatic radicals each of at least 10 carbon atoms); of these, the monoselenides are ordinarily preferred.

Suitable organo groups, which are preferably hydrocarbon groups, include alkyl groups, such as decyl, lauryl, cetyl, etc., alkylated cycloaliphatic radicals, such as ethyl cyclohexyl, dimethyl cyclohexyl, etc., alkylated aralykyl radicals, such as cetylbenzyl, butylbenzyl, etc., and the aliphatic radicals derived from halogenated mixtures of hydrocarbons such as chlorinated naphtha, chlorinated kerosene, chlorinated paraffin wax, etc. The aliphatic groups may contain non-hydrocarbon substituents such as chlorine, bromine, hydroxyl and amino so long as their essentially hydrocarbon character remains substantially unchanged. Of these various types of organo groups, the alkyl radicals are preferred and of these, the dodecyl group is especially preferred.

The cationic salt-forming radical may be metals, such as sodium, calcium, barium, zinc, potassium, lithium, strontium, aluminum, lead, thallium, etc., or the ammonium radical. Preferably, the metals are the polyvalent metals, especially those of Groups IIb, IV and VIII of the periodic table.

The following specific examples of selenides will further illustrate the selenium compounds of the present invention: dialkyl selenides, such as octyl decyl monoselenide, dilauryl monoselenide, di-eicosyl monoselenide, dialkyl diselenides, such as didecyl diselenide, didodecyl diselenide (dilauryl diselenide), diheptadecyl diselenide, dieicosyl diselenide, selenomercaptans, such as lauryl selenomercaptan, cetyl selenomercaptan, octadecyl selenomercaptan, paraffin wax selenomercaptan, etc., and the corresponding sodium, calcium, barium, zinc, cadmium and lead salts of such selenomercaptans.

Suitable base oils include a wide variety of lubricating oils such as naphthenic base, paraffin base, and mixed base mineral oils, other hydrocarbon lubricants, e. g., lubricating oil derived from coal products, and synthetic oils, e. g., alkylene polymers (such as polymers of propylene, butylene, etc., and mixtures thereof), alkylene oxide-type polymers, dicarboxylic acid esters and liquid esters of acids of phosphorus. Synthetic oils of

the alkylene oxide-type polymer which may be used include those exemplified by the alkylene oxide polymers (e. g., propylene oxide polymers) and derivatives, including alkylene oxide polymers prepared by polymerizing alkylene oxides, e. g., propylene oxide, in the presence of water or alcohols, e. g., ethyl alcohol, and esters of alkylene oxide-type polymers, e. g., acetylated propylene oxide polymers prepared by acetylating propylene oxide polymers containing hydroxyl groups.

Synthetic oils of the dicarboxylic acid ester type include those which are prepared by esterifying such dicarboxylic acids as adipic acid, azelaic acid, suberic acid, sebacic acid, alkyl succinic acid (such as those described in Moser Patents 2,124,628 and 2,133,734), fumaric acid, maleic acid, etc., with alcohols such as butyl alcohol, hexyl alcohol, 2-ethyl-hexyl alcohol, dodecyl alcohol, etc. Examples of dicarboxylic acid ester synthetic oils include dibutyl adipate, dihexyl adipate, di-2-ethyl-hexyl sebacate, di-n-hexyl fumarate polymer, etc.

Synthetic oils of the type of liquid esters of acids of phosphorus include the esters of phosphoric acid, e. g., tricresyl phosphate; the esters of phosphonic acid, e. g., diethyl ester of decane phosphonic acid.

Other suitable phosphonic acid esters may be obtained by the process described in Jensen and Clayton application Serial No. 86,856 filed April 11, 1949, now abandoned, according to which process hydrocarbons containing at least one aliphatic carbon atom are exposed simultaneously to the action of phosphorus trichloride and an oxygen-containing gas to produce hydrocarbon phosphonyl chlorides which may be converted to the desired esters, such as reacting the alkyl phosphonyl chloride with hydroxyl-containing compounds such as phenols and aliphatic alcohols or with olefin oxides such as propylene oxide or the like.

The oxidation inhibitors (i. e., the organic selenium compounds) which are present in the lubricating oil composition may be present in amounts from about 0.0001% to about 5% by weight of the final composition, that is, an amount sufficient to increase the resistance of the lubricating oil composition to oxidation. It is preferred to use from about 0.1% to about 2.0%.

The hydroxyanthraquinones of this invention (e. g., quinizarin) may be present in the final mineral oil composition in amounts from about 0.0001% to about 1.0% by weight of the final composition. It is preferred to use an amount sufficient to enhance the oxidation-inhibiting characteristics of the organic selenium compound, preferably from about 0.02% to about 0.1%.

The organic selenium compound may be replaced in part by alkylated phenol oxidation inhibitors, such as 2,6-di-tertiary butyl-4-methyl phenol, to procure a long life for the compounded oil. This is desirable since it provides a way of cutting down the amount of expensive selenide without reducing the long life as obtainable with selenides alone. Thus, a hydroxyanthraquinone (e. g., quinizarin) may be added to a lubricating oil containing an alkylated phenol oxidation inhibitor (e. g., 2,6-di-tertiary butyl-4-methyl phenol) and a selenide oxidation inhibitor (e. g., dilauryl monoselenide) to obtain a long life for the compounded oil.

A remarkable feature of this invention is the wholly unexpected, greatly enhanced synergistic effects which are obtained between lubricating oil oxidation inhibitors (e. g., organic selenium compounds) and the hydroxy anthraquinones (e. g.,

quinizarin). Nowhere would any one expect to find such synergistic effects as disclosed herein by the addition of a hydroxyanthraquinone as a secondary agent to a lubricating oil composition containing additives which are known to inhibit oxidation, particularly to find its anti-oxidation properties enhanced so tremendously by the addition of a secondary agent which in itself has relatively no effect in inhibiting oxidation in a lubricating oil. Obviously, it is not merely an additive effect which is obtained between the combinations of the known oxidation inhibitor in the lubricating oil and the hydroxyanthraquinones because the hydroxyanthraquinones in themselves are practically ineffective in inhibiting the oxidation in the lubricating oil composition.

In the tables hereinbelow, data are presented to show the synergistic effects obtained by testing the compositions of additives in a lubricating oil under severe conditions. In order to test effectively the compositions of this invention, a more drastic test was devised than is normally used in evaluating transformer oils and the like. This test has been called the California Research Transformer Oil Stability Test. The test is run as follows:

A 300-gram sample to be tested is placed in a glass tube which is set in an oil bath at 250° F. Oxidation catalysts, i. e., 112½ square centimeters of medium silicon transformer iron (such as USS Trancor 72) and 450 square centimeters of No. 14 gauge ASTM electrolytic copper wire are inserted in the tube. Oxygen is bubbled through the test sample at the rate of 3 liters per hour until the test sample has an acid number of 1.0 (milligrams of KOH per gram sample of oil). The number of hours required for the sample to show an acid number of 1.0 is known as the "test life" of the sample.

The data presented in the following tables will serve to illustrate the nature of the results that were obtained in accordance with the present invention.

Table I.—Quinizarin in a mineral oil containing dilauryl selenide

| Test No. | Oil                   | Additive (Percent by Weight) |            | Test Life (Hours) |
|----------|-----------------------|------------------------------|------------|-------------------|
|          |                       | Dilauryl Mono-selenide       | Quinizarin |                   |
| 1        | Base Oil <sup>1</sup> |                              |            | 24                |
| 2        | do <sup>1</sup>       |                              | 0.3        | 24                |
| 3        | do <sup>1</sup>       | 0.3                          |            | 115               |
| 4        | do <sup>1</sup>       |                              | 0.05       | 25                |
| 5        | do <sup>1</sup>       | 0.3                          | 0.05       | 365               |
| 6        | do <sup>2</sup>       |                              |            | <24               |
| 7        | do <sup>2</sup>       |                              | 0.05       | 25                |
| 8        | do <sup>2</sup>       | 0.3                          |            | 90                |
| 9        | do <sup>2</sup>       | 0.3                          | 0.05       | 465               |
| 10       | do <sup>3</sup>       |                              |            | <24               |
| 11       | do <sup>3</sup>       |                              | 0.05       | 20                |
| 12       | do <sup>3</sup>       | 0.3                          |            | 200               |
| 13       | do <sup>2</sup>       | 0.3                          | 0.05       | 355               |

<sup>1</sup> A California solvent-refined paraffinic base oil having a viscosity of 58 SSU at 100° F., and having 90% unsulfonatable residue.

<sup>2</sup> The base oil of (1) which had been treated further to yield an oil having 95% unsulfonatable residue.

<sup>3</sup> The base oil of (1) which had been treated further to yield an oil having 98% unsulfonatable residue.

Table II hereinbelow presents data on the results obtained by replacing in part and in toto dilauryl selenide (in a lubricating oil composition containing quinizarin) with 2,6-di-tertiary butyl-4-methyl phenol.

Table II.—Quinizarin in a mineral oil containing dilauryl monoselenide and/or 2,6-di-tertiary butyl-4-methyl phenol

| Test No. | Oil                   | Additive (Percent by Weight) |                                       |            | Test Life (Hours) |
|----------|-----------------------|------------------------------|---------------------------------------|------------|-------------------|
|          |                       | Dilauryl Mono-selenide       | 2,6-Di-tertiary Butyl-4-Methyl Phenol | Quinizarin |                   |
| 10       | Base Oil <sup>1</sup> |                              |                                       |            | 24                |
| 14       | do <sup>1</sup>       |                              |                                       | 0.05       | 25                |
| 15       | do <sup>1</sup>       |                              | 0.3                                   |            | 70                |
| 16       | do <sup>1</sup>       | 0.3                          |                                       |            | 115               |
| 17       | do <sup>1</sup>       | 0.3                          |                                       | 0.05       | 365               |
| 18       | do <sup>1</sup>       | 0.3                          |                                       | 0.05       | 310               |
| 19       | do <sup>1</sup>       | 0.2                          | 0.1                                   | 0.05       | 490               |
| 20       | do <sup>1</sup>       |                              |                                       |            | <24               |
| 21       | do <sup>1</sup>       |                              | 0.3                                   |            | 95                |
| 22       | do <sup>1</sup>       |                              | 0.3                                   |            | 20                |
| 23       | do <sup>2</sup>       |                              |                                       | 0.05       | 325               |
| 24       | do <sup>2</sup>       |                              | 0.3                                   | 0.05       | <24               |
| 25       | do <sup>3</sup>       |                              |                                       | 0.05       | 20                |
| 26       | do <sup>3</sup>       |                              | 0.3                                   |            | 175               |
| 27       | do <sup>3</sup>       |                              | 0.3                                   | 0.05       | 400               |

<sup>1</sup> A California solvent-refined paraffinic base oil having a viscosity of 58 SSU at 100° F., and having 90% unsulfonatable residue.

<sup>2</sup> The base oil of (1) which had been treated further to yield an oil having 95% unsulfonatable residue.

<sup>3</sup> The base oil of (1) which had been treated further to yield an oil having 98% unsulfonatable residue.

The data of above Table II show that the "test life" of a lubricating oil containing a dialkyl monoselenide oxidation inhibitor and an alkylated phenol oxidation inhibitor is remarkably increased by incorporating therein a hydroxyanthraquinone. These data show that the combination of a hydroxyanthraquinone (e. g., quinizarin), a selenide oxidation inhibitor (e. g., dilauryl monoselenide), and an alkylated phenol oxidation inhibitor (e. g., 2,6-di-tertiary butyl-4-methyl phenol) in a lubricating oil exhibits a remarkable synergistic effect to enhance the anti-oxidation characteristics of the lubricating oil composition.

In some instances, 2,6-di-tertiary butyl-4-methyl phenol and similar alkylated phenol oxidation inhibitors may replace in toto the selenide oxidation inhibitor. That is, a hydroxy anthraquinone (e. g., quinizarin) may be added to a lubricating oil containing an alkylated phenol oxidation inhibitor (e. g., 2,6-di-tertiary butyl-4-methyl phenol) to produce synergistic effects in prolonging the life of a lubricating oil composition.

Organic-tin compounds, such as tetraphenyl tin, are also effective to replace, in part, a portion of the organic selenium compounds (e. g., dilauryl monoselenide) which is present in a lubricating oil in combination with a hydroxyanthraquinone (e. g., quinizarin). Furthermore, a hydroxyanthraquinone is effective for increasing the life of a lubricating oil containing an alkylated phenol oxidation inhibitor (e. g., 2,6-di-tertiary butyl-4-methyl phenol) in combination with an organo-tin compound (e. g., tetraphenyl tin). For example, when 0.1% by weight of 2,6-di-tertiary butyl-4-methyl phenol and 0.06% by weight of tetraphenyl tin are incorporated in a California solvent-refined paraffinic base oil having a viscosity of 58 SSU at 100° F. containing 0.05% quinizarin, the life of the base oil was increased from 24 hours to greater than 1000 hours.

The combination of additives of the present invention may be used effectively in oils generally, whether hydrocarbon or non-hydrocarbon, although their present field of chief utility is in transformer oils and in turbine oils. The hydroxy-anthraquinones may also be used in oils

containing other groups of additives in addition to anti-oxidants. For example, in addition to the above-noted compounds, the lubricating oils may contain other agents, such as pour point depressants, oiliness agents, extreme pressure agents, blooming agents, compounds for enhancing the viscosity index of the hydrocarbon oil, grease-forming agents, peptizing agents, etc.

We claim:

1. A transformer oil composition consisting essentially of a major portion of an oil of lubricating viscosity and from about 0.0001% to about 5%, by weight, of a dialkyl monoselenide containing from 12 to 30 carbon atoms in each alkyl group, to which transformer oil composition is added from about 0.000% to about 1.0%, by weight, of a hydroxy anthraquinone selected from the group consisting of 1,2-dihydroxy-anthraquinone; 1,4-dihydroxy-anthraquinone; 1,5-dihydroxy-anthraquinone and 1,8-dihydroxy-anthraquinone.

2. A transformer oil composition consisting essentially of a major portion of an oil of lubricating viscosity and from about 0.1% to about 2.0%, by weight, of a dialkyl monoselenide containing from about 12 to 30 carbon atoms in each alkyl group, to which transformer oil composition is added from about 0.02% to about 1.0%, by weight,

8  
of a hydroxy anthraquinone selected from the group consisting of 1,2-dihydroxy-anthraquinone; 1,4-dihydroxy-anthraquinone; 1,5-dihydroxy-anthraquinone and 1,8-dihydroxy-anthraquinone.

3. The transformer oil composition of claim 1, wherein said oil is a petroleum lubricating oil.

4. The transformer oil composition of claim 1, wherein the dialkyl monoselenide is di-lauryl monoselenide.

5. The transformer oil composition of claim 1, wherein the dihydroxy-anthraquinone is quinizarin.

WILLIAM T. STEWART.  
CHARLES D. NEWNAN.  
NEAL W. FURBY.

References Cited in the file of this patent

UNITED STATES PATENTS

| Number    | Name           | Date           |
|-----------|----------------|----------------|
| 2,016,648 | Orelup         | Oct. 8, 1935   |
| 2,053,421 | Burk et al.    | Sept. 8, 1936  |
| 2,214,443 | Varteressian   | Sept. 10, 1940 |
| 2,225,533 | Dewey          | Dec. 17, 1940  |
| 2,261,888 | Rocchini       | Nov. 4, 1941   |
| 2,398,415 | Denison et al. | Apr. 16, 1946  |